# EUROPEAN PATENT APPLICATION

(11) **EP 2 618 337 A2**
(43) Date of publication of application: **24.07.2013**
(21) Application number: 13164535.0
(22) Date of filing: 09.03.2011
(51) Int. Cl.: H01B 7/295

(54) **Conductor insulation with micro oxide particles**

(30) Priority: 12.03.2010 US 313513 P; 06.04.2010 US 321360 P
(62) Divisional of application: 11754001.3
(71) Applicant: General Cable Technologies Corporation, Highland Heights KY 41076 (US)
(72) Inventor: Szylakowski, Gregg, Loveland, OH 45140 (US); Albrinck, Alice, Hebron, KY 41048 (US); McLinn, Matthew S., Cincinnati, OH 45202 (US)
(74) Representative: Lowe, Alastair Nicholas

(57) **Abstract**

An insulated conductor, comprising
a conductor; and
at least one layer of a composite insulation surrounding said conductor, said composite insulation including insulating material and micro oxide particles adapted to provide at least one of an increase in the flame retardancy of the insulating material and an improvement in the electrical properties of the insulating material.

## Description

### Related Application

This application claims priority to U.S. Provisional Application Serial No. 61/313,513, filed on March 12, 2010, and U.S. Provisional Application Serial No. 61/321,360, filed on April 6, 2010, both entitled Insulation With Micro Oxide Particles and Cable Using the Same.

### Field of the Invention

The present invention relates to insulation with micro oxide particles. More specifically, the present invention relates to insulation and cable jackets with micro oxide particles used with cable and cable components for increasing the flame retardancy and the electrical performance of the cable.

### Background of the Invention

Wire and cable insulation or coating or component compositions are normally quite flammable. As a result, they can pose a fire hazard in power plants, distribution areas, manholes, and buildings. Ignition can easily occur from overheating or arcing. Accordingly, various fire codes prohibit the use of cables, particularly in plenum applications, unless they pass certain smoke and flame retardancy tests. Therefore, flame retardants are generally used tin wire and cable insulation and coatings to prevent electric sparks and subsequently to prevent the spread of fire alone the cable.

Flame retardants, such as halogenated additives (compounds based on fluorine, chloring or bromine) or halogenated polymers, such as chlorosulfonated polyethylene, neoprene, polyvinyl chloride, or the like, are commonly used in wire and cable insulation or coating compositions. Both halogenated additives and halogenated polymers are capable of giving fire-resistant properties to the polymer that forms the coating. Halogens, however, have a drawback in that the gases evolved (i.e. hydrogen chloride, hydrogen fluoride and hydrogen bromide) during burning, or even merely overheating, are corrosive as well as being toxic which is often limited by building codes or undesirable in some building overheating locations.

Another alternative for providing flame retardancy for wire and cable insulation is to use a metal hydroxide, which is inorganic, hydrated, and porous, as a filler in the polymer matrix. The metal hydroxide provides flame retardancy by a mechanism known as water of hydration. When the metal hydroxide is heated, water is evolved which effects a flame retardant action. A drawback of this system is that the metal hydroxide is polar, which absorbs moisture when the cable is exposed to a wet environment, resulting in a reduction in the electrical insulation properties of the coating composition. Use of metal hydroxides also limits processing temperature of the insulation.

Plenum rated cables are often made from various fluoropolymer materials, such as fluoroethylenepropylene (FEP), to provide flame retardancy. However, such fluoropolymer materials are expensive and significantly increase manufacturing costs. Also, FEP has been found to produce smoke under high or intense heat conditions which is often undesirable in building overheating locations.

Some fillers, such as calcium carbonates and kaolins, have been added to insulation; however such fillers are hydrophilic, increase the dissipation factor of the insulation, lower the dielectric constant of the insulation, thereby causing greater attenuation and delay skew. Delay is the time it takes a signal to travel the length of a pair. Delay skew is the difference between the longest and shortest delay among the pairs in the cable. Other fillers, such as glass, have been attempted; however the glass contains large amounts of sodium sulfate, sodium chloride, boron, iron and/or calcium that increase the insulation's dissipation factor. When the dissipation factor of the insulation is increased, the dielectric constant of the insulation is lower, thereby causing greater attenuation and delay skew. This increase in dissipation factor of the insulation cause greater attenuation of the signal along the length of the transmission line. Multiplatlet clays that are treated with ionic or cationic exfoliating agents have also been added to insulation, however such additives cause undesirable dielectric properties, they impart stiffness when cables are usually desired to be flexible, and their high surface areas cause undesirable rheological properties, such as increased viscosity, thereby limiting the amounts that can be added to the insulation.

### Summary of the Invention

According to an exemplary embodiment, the present invention provides a composite insulation that includes an insulating material and amorphous micro oxide particles added to the insulating material by at least 1% weight of the composition insulation wherein the micro oxide particles increase the flame retardancy and/or electrical properties of the insulating material of a cable jacket or bedding or other cable component such as a separator, for example. In one embodiment, the micro oxide particles are silicon dioxide. The composite of the invention can advantageously be used on power, data, communication, control, safety, transit, military, automotive, shipboard or other types of cable.

According to another embodiment, the present invention provides a composite insulation, jacket, bedding or other cable component that comprises an essentially solid non-porous low surface area, non-ionic, non-hydrated, mineral or metal micro oxide particles.

According to another exemplary embodiment, the present invention provides an insulated conductor including a conductor and at least one layer of a composite insulation surrounding the conductor. The composite insulation includes insulating material and micro oxide particles adapted to increase the flame retardancy and/or electrical properties of the insulation material. In one embodiment, the micro oxide particles are silicon dioxide.

According to yet another exemplary embodiment, the present invention provides a cable that includes at least a first pair of conductors where at least one of the first pair of conductors has at least one layer of a composite insulation surrounding the conductor. The composite insulation includes insulating material and micro oxide particles adapted to increase the flame retardancy or electrical properties of the insulation material, whereby the conductors of the first pair of conductors may be either twisted together or not twisted together.

According to still another exemplary embodiment, the present invention provides a cable comprising a plurality of conductors where each conductor is surrounded by a layer of insulating material. A jacket encloses the plurality of conductors and the jacket is formed of an insulating material. A separator separates the plurality of conductors and the separator is formed of an insulating material. The insulation material of at least one of the plurality of conductors, the jacket, and the separator includes micro oxide particles to form a composite insulation which has an increased flame retardancy over the insulation material without the micro oxide particles.

According to still another exemplary embodiment, the present invention provides a cable comprising a plurality of conductors where each conductor is surrounded by a layer of insulating material. A jacket encloses the plurality of conductors. A bedding compound surrounds the plurality of conductors and fills the gaps underneath the jacket. The insulation material of at least one of the plurality of conductors and or the jacket, and or the bedding includes micro oxide particles to form a composite which has an increased flame retardancy over the cable without the micro oxide particles.

Other objects, advantages and salient features of the invention will become apparent from the following detailed description, which, taken in conjunction with the annexed drawings, discloses a preferred embodiment of the present invention.

### Brief Description of the Drawings

A more complete appreciation of the invention and many of the attendant advantages thereof will be readily obtained as the same becomes better understood by reference to the following detailed description when considered in connection with the accompanying drawings, wherein:

FIG. 1 is a cross sectional view of a cable in accordance with an exemplary embodiment of the present invention; and

FIG. 2 is a cross section view of conductor pairs with more than one layer of insulation in accordance with an exemplary embodiment of the present invention.

### Detailed Description of the Invention

Referring to Figures 1 and 2, the present invention generally relates to a composite insulation for cable and its components that includes added non-porous micro oxide particles to improve the flame retardancy and electrical performance characteristics of the cable while also reducing costs. For example, with the addition of the non-porous micro oxide particles to the insulation, the insulation has (a) a decreased melt flow rate that contributes to a reduction in dripping, i.e. the melt flow index is decreased by up to about 100 %, preferably about 3-50%, thereby decreasing the risk of flame spread and exhibiting less smoke when exposed to flame; (b) an increased dielectric constant by about 2-50%, and preferably 3-30%, thereby refining electrical performance; (c) an increased viscosity by 3-100%, preferably by about 3-30%, which improves and simplifies extruding; (d) preferably about 30-100% less transparency so that less, if any, coloring agent is required, to make the insulating material, cable jacket, bedding or other cable component opaque, and also produces brighter colors; and (e) increased charring by preferably about 3-30%, which results in more char and less burned or melted material which would give off smoke and chemicals. By adding micro oxide particles in the insulation, such as FEP for example, less FEP is required to achieve the same or better burn characteristics as conventional cable using only fluoropolymers. Alternatively, the micro oxide particles may be added to less expensive materials, such as polyethylene, to improve flame retardancy and electrical properties, and to reduce smoke generation.

Regarding the increased dielectric constant, the dielectric constant of an insulating compound considerably affects how that insulated wire or conductor and the resulting pair behaves electrically. FEP or fluorinated ethylene propylene, for example is not flammable, but instead drips and exudes smoke. When a cable containing FEP is subjected to the NFPA 262 test the dripping results in smoking material at the bottom of the chamber causing the optical density to increase. It has been demonstrated that higher melt flow FEP exhibits more dripping than lower melt flow FEP. FEP is excellent for use as a dielectric as it has an excellent dielectric constant of 2.1 and dissipation factor of 0.0005. Its low dielectric constant is essentially constant throughout various frequencies. FEP has excellent resistance to thermal and oxidative aging. FEP is considered to be one of the most chemical resistant polymers. FEP has a continuously effective usable temperature range from about -200°C to +200°C. Its boundaries inherently set the electrical limits for two important electrical characteristics in a cable: capacitance and velocity of propagation. Capacitance is affected in that increasing the dielectric constant of the insulation material, such as by mixing FEP and the micro oxide particles, such as spherically-shaped amorphous silicon dioxide micro particles, with respect to virgin FEP, increases its conductor pair's capacitance. See TABLE 1 below. This is advantageous where the insulation diameters arc fixed, impedance can be optimized by using an insulation material with a favorable dielectric constant, as impedance is very closely related to its capacitance. Secondly, a pair's dielectric constant affects the velocity of propagation of its electrical signal. By increasing the dielectric constant of the insulation material, such as by mixing FEP and the micro oxide particles/silicon dioxide with respect to virgin FEP, the resulting pair comparably slows down the transmitted signal. This phenomenon is advantageous in the case of a design of a cable with two different insulation types because it brings the delay skew of the cable closer together. This has been a restrictive constraint in the design of prior art cables.

**TABLE 1**

| **Sample ID** | **Frequency** | **Dielectric Constant** | **Dissipation Factor** |
|---|---|---|---|
| 0% Sidistar/100% FEP | 1 kHz | 2.039 | 0.00222 |
| | 1 MHz | 2.038 | 0.0004 |
| | 10 MHz | 2.031 | 0.00252 |
| 5% Sidistar/95% FEP | 1 kHz | 2.109 | 0.00189 |
| | 1 MHz | 2.105 | 0.00078 |
| | 10 MHz | 2.099 | 0.00249 |
| 10% Sidistar/90% FEP | 1 kHz | 2.185 | 0.00236 |
| | 1 MHz | 2.18 | 0.00079 |
| | 10 MHz | 2.173 | 0.00274 |
| 15% Sidistar/85% FEP | 1 kHz | 2.268 | 0.00258 |
| | 1 MHz | 2.26 | 0.00102 |
| | 10 MHz | 2.254 | 0.00285 |
| 20% Sidistar/80% FEP | 1 kHz | 2.353 | 0.00275 |
| | 1 MHz | 2.343 | 0.00111 |
| | 10 MHz | 2.338 | 0.00262 |
| 25% Sidistar/75% FEP | 1 kHz | 2.441 | 0.00303 |
| | 1 MHz | 2.428 | 0.00119 |
| | 10 MHz | 2.423 | 0.0017 |

The amorphous silicon dioxide was added into high density polyethylene (HDPE) at various loading levels (5%, 10%, 15%, 20% and 25%). TABLE 2 shows the resulting materials and their dielectric and dissipation characteristics. As the silicon dioxide loading level increases, so does the dielectric constant across all tested frequencies, although by a lower rate than it did in FEP. The dissipation factor is also fairly consistent among all loading levels. In addition to electrical properties, observations were made to the behavior of the samples as they were burned. With the addition of silicon dioxide to the HDPE, the flame spread traveled at a slower rate as the percentage of silicon dioxide increased. The materials also had reduced dripping as compared to the standard material. It is preferred that a cable be manufactured using a 25% loading of silicon dioxide into HDPE.

**TABLE 2**

| **Loading Percentage** | **Frequency** | **Dielectric Constant** | **Dissipation Factor** |
|---|---|---|---|
| 0% Sidistar/100% HDPE | 1 kHz | 2.296 | 0.00326 |
| | 1 MHz | 2.313 | 0.00127 |
| | 10 MHz | 2.300 | 0.06410 |
| 5% Sidistar/95% HDPE | 1 kHz | 2.325 | 0.00346 |
| | 1 MHz | 2.343 | 0.00155 |
| | 10 MHz | 2.329 | 0.06560 |
| 10% Sidistar/90% HDPE | 1 kHz | 2.353 | 0.00347 |
| | 1 MHz | 2.373 | 0.00125 |
| | 10 MHz | 2.357 | 0.06750 |
| 15% Sidistar/85% HDPE | 1 kHz | 2.389 | 0.00299 |
| | 1 MHz | 2.404 | 0.00119 |
| | 10 MHz | 2.391 | 0.05640 |
| 20% Sidistar/80% HDPE | 1 kHz | 2.425 | 0.00361 |
| | 1 MHz | 2.443 | 0.00162 |
| | 10 MHz | 2.428 | 0.06510 |
| 25% Sidistar/75% HDPE | 1 kHz | 2.459 | 0.00322 |
| | 1 MHz | 2.474 | 0.00155 |
| | 10 MHz | 2.461 | 0.06000 |

The amorphous silicon dioxide was added into ethylene vinyl acetate (EVA) at various loading levels (5%, 10%, 15%, 20% and 25%). TABLE 3 shows the resulting materials and their dielectric and dissipation characteristics.

**TABLE 3**

| **Loading Percentage** | | | |
|---|---|---|---|
| | **Frequency** | **Dielectric Constant** | **Dissipation Factor** |
| 0% Sidistar / 100% EVA | 1 kHz | 2.903 | 0.0042 |
| | 1 MHz | 2.703 | 0.0345 |
| | 10 MHz | 2.530 | 0.0387 |
| 10% Sidistar / 90% EVA | 1 kHz | 2.927 | 0.0009 |
| | 1 MHz | 2.738 | 0.0322 |
| | 10 MHz | 2.577 | 0.0356 |
| 20% Sidistar / 80% EVA | 1 kHz | 3.031 | 0.0075 |
| | 1 MHz | 2.826 | 0.0307 |
| | 10 MHz | 2.661 | 0.0345 |
| 30% Sidistar / 70% EVA | 1 kHz | 3.042 | 0.0077 |
| | 1 MHz | 2.858 | 0.0276 |
| | 10 MHz | 2.714 | 0.0306 |
| 40% Sidistar / 60% EVA | 1 kHz | 3.159 | 0.0091 |
| | 1 MHz | 2.967 | 0.0261 |
| | 10 MHz | 2.827 | 0.0288 |
| 50% Sidistar / 50% EVA | 1 kHz | 2.977 | 0.0111 |
| | 1 MHz | 3.180 | 0.0235 |
| | 10 MHz | 2.954 | 0.0275 |
| 60% Sidistar / 40% EVA | 1 kHz | 2.985 | 0.0117 |
| | 1 MHz | 3.268 | 0.0193 |
| | 10 MHz | 3.046 | 0.0220 |

The increased viscosity resulting from adding the micro oxide particles to the insulation, as seen in the graph below, improves the processing characteristics of fluoropolymers and other pseudo plastic polymers during the extrusion process. Tip and die drool are minimized in fluoropolymers and other polymers utilized in the invention. Inherent fluoropolymer processing issues, such as disruptions in consistent material flow (commonly referred to as cone pulsations), result in knots or lumps (diameter fluctuations). FEP, for example, exhibits strongly pseudo plastic behavior making it difficult to extrude at higher speeds and higher shear rates. Low pressure in the die causes instability in extrusion and uneven wall thickness, cone pulsations, knots or lumps. The composition of the invention and its resulting increased viscosity minimizes flow disruptions and the associated defects. The increased viscosity is about 3 -100%. The exact amount of viscosity increase desired will depend on the viscosity or MFi of the polymer used. Lower MFi, higher viscosity polymers may be used, however such polymers may be higher in cost, exhibit less shear thinning, be highly viscoelastic, cause breaks in the insulation or have les desirable dielectric properties. The invention allows selection of the optimum polymer and the ability to tailor its viscosity. It permits the ability to utilize pressure tooling versus tube tooling to increase line speeds or manufacturing rates.

According to an exemplary embodiment of the invention, the micro oxide particles are oxides of a non-ionic, i.e. without a positive or negative ionic valence, cannot form an ionic bond, mineral or metal (element). Preferably the particles have a low surface area that impart improved dielectric, rheological, and fire resistance properties. The surface area of the micro oxide particles is preferably about 10 - 40m²/g. Preferred oxides include Silicon, Aluminum, Magnesium and their double oxides. Zn and Fe oxides may also be suitable for some embodiments of the invention. Other oxides are envisioned to function in the invention but may not yet be available in the micro form described in the invention. Also, the micro oxide particles are preferably solid non porous amorphous particles, i.e. not crystalline material. The particle size of the micro oxide particles may be less than 0.300 µm, and is preferably in the range of 0.100 - 0.300 µm. The concentration of the micro oxide particles may be about 1 to 80% by weight of the insulation, and is preferably about 2-50%, and most preferred about 3-25%.

A preferred micro oxide particle is SIDISTAR® T 120, made by Elkem Silicon Materials, which is a spherically-shaped amorphous silicon dioxide additive designed for polymer applications. The average primary particle size of SIDISTAR® T 120 is 150nm. Depending on the selected polymer, the SIDISTAR® T120 additive provides increased flame retardancy, greater stiffness, improved melt flow, improved surface finish, improved melt strength, improved dryblend flow, impact strength, and lower cost. In the mixing process, SIDISTAR® T120 improves the dispersion of all compound ingredients, providing well-balanced physical properties in the final insulation. Because it is dispersed as primarily spherical particles, it reduces internal friction and allows higher extrusion or injection speed as the result of better melt flow and therefore significant cost savings. Dispersion down to primary particles within the matrix enables a very fine cell formation, resulting in a reduction of high molecular weight processing aid and therefore much reduced raw material costs. Table 4 below provides the product specification of SIDISTAR® T 120.

**TABLE 4**

| **Properties** | **Unit** | **Limits** |
|---|---|---|
| SiO₂ (Silicon dioxide, amorphous) | % | 96,0-99,0 |
| C (Carbon) | % | ≤0.20 |
| Fe₂O₃ (Iron oxide) | % | ≤0.25 |
| H₂O | % | ≤ 0.8 |
| Loss on Ignition (L.O.I.) @ 950°C | % | ≤ 0.60 |
| Coarse Particles (325 mesh) | % | ≤ 0.10 |
| pH-value | | 7.0 - 9.0 |
| Bulk Density | kg/m³ | 400 - 700 |
| Specific Surface Area (BET) | m²/g | 20 |
| L-value | % | ≥ 89.5 |
| Median particle size | µm | 0.15 |
| Density | g/cm³ | 2.2 |

Other materials, such as silica fume, may be used as the micro oxide particles. Silica fume is also called microsilica Silica and is a byproduct in the reduction of high-purity quartz with coke in electric arc furnaces during the production of silicon and ferrosilicon. Silica fume consists of fine vitreous particles with a surface area of about 20m²/g, with particles approximately 0.150mm (micro meters) in diameter. The silica fume improves reology characteristics of the composite insulation.

Any polymer or thermoplastic known in the cable art may be used as the main component of the composite insulation to which the micro oxide particles may be added. For example, the insulation may be polyolefin, polyester, fluoropolymer, Halar, PTFE, PVC, and the like.

The polyethylene may be of the various types known in the art. Low density polyethylene ("LDPE") can be prepared at high pressure using free radical initiators, or in gas phase processes using Ziegler-Natta or vanadium catalysts, and typically has a density in the range of 0.914 - 0.940 g/cm³. LDPE is also known as "branched" or "heterogeneously branched" polyethylene because of the relatively large number of long chain branches extending from the main polymer backbone. To reduce the density of such high density polyethylene resins below the range of densities that are normally produced in such processes, another alpha-olefin or co-monomer, may be copolymerized with the ethylene. If enough co-monomer is added to the chain to bring the density down to 0.912-0.939 gram/cc, then such products are known as linear, low density polyethylene copolymers. Because of the difference of the structure of the polymer chains, branched low density and linear, low density polyethylene have different properties even though their densities may be similar.

It will be understood that the term "linear low density polyethylene" is meant to include copolymers of ethylene and at least one alpha-olefin comonomer. The term includes copolymers, terpolymers, and the like. Linear low density polyethylenes are generally copolymers of ethylene and alpha-olefins, such as propene, butene, 4-methyl-pentene, hexene, octene and decene.

Polyethylene in the same density range, i.e., 0.916 to 0.940 g/cm³, which is linear and docs not contain long chain branching may also be used. This "linear low density polyethylene" ("LLDPE") can be produced with conventional Ziegler-Natta catalysts or with metallocene catalysts. Relatively higher density LDPE, typically in the range of 0.928 to 0.940 g/cm³, is sometimes referred to as medium density polyethylene ("MDPE"), may also be used. Linear low density polyethylene copolymers may be prepared utilizing the process, for example, as described in U.S. Pat. Nos. 3,645,992 and 4,011,382, the disclosures of which are incorporated herein by reference. The co-monomer which is copolymerized with the polyethylene is preferably an alpha-olefin having from about 3 up to about 10 carbon atoms. The density of the ethylene copolymer is primarily regulated by the amount of the co-monomer which is copolymerized with the ethylene. In the absence of the co-monomer, the ethylene would homopolymerize in the presence of a stereospecific catalyst to yield homopolymers having a density equal to or above 0.95. Thus, the addition of progressively larger amounts of the co-monomer to the ethylene monomer, results in a progressive lowering, in approximately a linear fashion, of the density of the resultant ethylene copolymer.

Low density polyethylenes suitable for use in the present invention include ethylene homopolymers and copolymers having up to 20% (w/w) of a comonomer, such as vinyl acetate, butyl acrylate and the like.

Polyethylenes may be used having still greater density, such as the high density polyethylenes ("HDPEs"), i.e., polyethylenes having densities greater than 0.940 g/cm³, and are generally prepared with Ziegler-Natta catalysts. High density polyethylene resins, i.e., resins having densities ranging up to about 0.970 gram/cc are manufactured at lower pressures and temperatures via heterogeneous ionic catalytic processes, for example, those utilizing an organometallic or a transition metal oxide catalyst. The products are linear, non-branched polyethylene.

Very low density polyethylene ("VLDPE") may also be used. VLDPEs can be produced by a number of different processes yielding polymers with different properties, but can be generally described as polyethylenes having a density less than 0.916 g/cm³, typically 0.890 to 0.915 g/cm³ or 0.900 to 0.915 g/cm³.

U.S. Pat. Nos. 5,272,236 and 5,278,272, the subject matter of each of which is herein incorporated by reference, disclose polyethylenes termed "substantially linear ethylene polymers" ("SLEPs"). These SLEPs are characterized as having a polymer backbone substituted with about 0.01 long chain branches/1000 carbons to about 3 long chain branches/1000 carbons, more preferably from about 0.01 long chain branches/1000 carbons to about 1 long chain branches/1000 carbons, and especially from about 0.05 long chain branches/1000 carbons to about 1 long chain branches/1000 carbons. As used herein, a polymer with "long chain branching" is defined as one having a chain length of at least about 6 carbons, above which the length cannot be distinguished using ¹³C NMR spectroscopy. It is further disclosed that the long chain branch can be as long as about the same length as the length of the polymer backbone. As used in the present invention, the term "linear" is applied to a polymer that has a linear backbone and does not have long chain branching; i.e., a "linear" polymer is one that does not have the long chain branches characteristic of an SLEP polymer.

Preferably the polyethylenes selected for use in the compositions of the present invention have melt indices in the range of from 1 to 30g/600s, more preferably 2 to 20 g/600s. Preferably the low density polyethylenes have a density in the range of from 913 to 930 kg/m³, more preferably in the range of from 917 to 922 kg/m³.

The elastomer used in the base polymer in accordance with the present invention may also be selected from the group of polymers consisting of ethylene polymerized with at least one comonomer selected from the group consisting of C₃ to C₂₀ alpha-olefins and C₃ to C₂₀ polyenes. Generally, the alpha-olefins suitable for use in the invention contain in the range of about 3 to about 20 carbon atoms. Preferably, the alpha-olefins contain in the range of about 3 to about 16 carbon atoms, most preferably in the range of about 3 to about 8 carbon atoms. Illustrative non-limiting examples of such alpha-olefins are propylene, 1-butene, 1-pentene, 1-hexene, 1-octene and 1-dodecene.

Preferably, the elastomers are either ethylene/alpha-olefin copolymers or ethylene/alpha-olefin/diene terpolymers. The polyene utilized in the invention generally has about 3 to about 20 carbon atoms. Preferably, the polyene has in the range of about 4 to about 20 carbon atoms, most preferably in the range of about 4 to about 15 carbon atoms. Preferably, the polyene is a diene, which can be a straight chain, branched chain, or cyclic hydrocarbon diene. Most preferably, the diene is a non conjugated diene. Examples of suitable dienes are straight chain acyclic dienes such as: 1,3-butadiene, 1,4-hexadiene and 1,6-octadiene; branched chain acyclic dienes such as: 5-methyl-1,4-hexadiene, 3,7-dimethyl-1,6-octadiene, 3,7 -dimethyl-1,7-octadiene and mixed isomers of dihydro myricene and dihydroocinene; single ring alicyclic dienes such as: 1,3-cyclopentadiene, 1,4-cylcohcxadicnc, 1,5-cyclooctadiene and 1,5-cyclododecadiene; and multi-ring alicyclic fused and bridged ring dienes such as: tetrahydroindene, methyl tetrahydroindene, dicylcopentadiene, bicyclo-(2,2,1)-hepta-2-5-diene; alkenyl, alkylidene, cycloalkenyl and cycloalkylidene norbornenes such as 5-methylene-2morbornene (MNB), 5-propenyl-2-norbornene, 5-isopropylidene-2-norbornene, 5-(4-cyclopentenyl)-2-norbornene, 5-cyclohexylidene-2-norbomene, and norbornene. Of the dienes typically used to prepare EPR's, the particularly preferred dienes are 1,4-hexadiene, 5-ethylidene-2-norbornene, 5-vinyllidene-2-norbornene, 5-methylene-2-norbornene and dicyclopentadiene. The especially preferred dienes are 5-ethylidene-2-norbornene and 1,4-hexadiene.

Preferably, the elastomers have a density of below 0.91, more preferably below 0.9. In preferred embodiments of the invention, the elastomer comprises metallocene EP which is an EPR or EPDM polymer or ethylene butane or ethylene octene polymers prepared with metallocene catalysts. In embodiments of the invention, the base polymer may be metallocene EP alone, metallocene EP and at least one other metallocene polymer, or metallocene EP and at least one non-metallocene polymer as described below.

Stabilizers may be added to the composite insulation. Stabilizers may be used primarily for long term stability and moisture resistance under dielectric stress, specifically dielectric constant or specific inductive capacitance (SIC). These additives act to immobilize active ions to form salts that are insoluble in water at higher temperatures such as 75°C or 90°C. These ions are typically present in the ppm level and exist as impurities within various additives used within this embodiment. Examples of stabilizers include lead stabilizer additives, such as dibasic lead phthalate and red lead. A non-lead example is hydrotalcite. Dibasic lead phthalate is the preferred stabilizer.

Antioxidants may be added to the insulation composite to prevent oxidative degradation of the polymers. Antioxidants, such as hydroquinones, hindered-phenols, phosphites, thioesters, epoxies, and aromatic amines, may be used. The preferred antidoxidants used in wire and cable are hydroquinones and/or hindered-phenols. A common hydroquinone is 1,2dihydro-2,2,4 trimethyl quinoline. Examples of hindered-phenols are distearyl 3,3'thio-dipropionate (DSTDP), bis(2,4 di terbutyl) pentaerythritol diphosphite, tris(2,4 di-terbutyl) pentaerythritol diphosphite, tris(2,4 di-terbutyl phenyl) phosphite, zinc 2-mercaptotoluimidazole salt, 2,2' thiodiethyl bis-(2,5-diterbutyl-4hydroxyphenyl, 2,2'-thiobis-(6 terbutyl paracresol) and dilauryl 3,3' thio-dipropionate.

The polyolefin compositions can be vulcanized using traditional curing procedures, such as chemical, thermal, moisture, room temperature vulcanization (RTV) and radiation procedures. The curing agents employed in the present invention can be organic peroxides, dicumyl peroxide and bis(terbutylperoxy) diisopropylbenzene. The peroxides act by decomposing at the cure temperature to form free radicals which then abstract a hydrogen from adjacent polymer molecules allowing the polymers to bond covalently to each other. To select the curing agents it is necessary to take into account the decomposition temperatures of the agents, in order to avoid undesirable problems during the mixture and extrusion processes. The curing agent amounts and/or ratios to be used will be defined based on the type of application because depending on the increase of the curing agent content in the formula, the following properties will be improved and/or reduced.

The composite insulation of the present invention may include other flame retardants, such as halogenated additives (compounds based on fluorine, chlorine or bromine) or halogenated polymers, such as chlorosulfonated polyethylene, neoprene, polyvinyl chloride, or the like. Effervescents, for example a combination of poly(ethylene-co-acrylate), chalk and silicone elastomer. Silicon or silicon containing flame retardants. Phosphorus Phospate esters containing flame retardants. The compositions may include other flame suppressants inorganic hydrated metal oxide such as Alumina trihydrate or Magnesium hydroxide. Synergists such as Antimony oxide or ammonium phosphate may be used. Other smoke suppressants such as Zinc borate, Barium borate, Zinc stannate, Zinc sulfide or copper salts may be used. Advantageously the micro oxide particles of the invention can lower the amounts of these additives necessary or increase flame redundancy in combination with these additives.

Mixing can be done by any method well know in the art including by internal mixers, twin screw extruders, kneaders, ribbon blenders, hi shear blade mixers and the like or even at the cable making extruders. A master batch can also first be made and let down by further mixing or used at the cable making extruder.

The composite material is then taken to an extruder. The material is fed through a hopper and carried down the length of a screw in the extruder, and forced through a crosshead die. At the same time, a conductor passes through the crosshead die where the molten coating material is applied around the conductor. This wire then goes through a cooling process, or if cross linking is desired a continuous vulcanization steam tube. At the end of the tube, the wire is reeled off and packaged.

In the case of multiconductor cable, a second insulated conductor is stranded or braided on to the reeled off wire. The cable is then passed through the crosshead die a second time where the outer coating is applied it can be vulcanized if desired.

### Testing (Drip)

The composite insulation of the present invention also provides improved dripping characteristics as demonstrated by the following testing of Standard 25 MFi 2.15 S.G. FEP produced by Daikin Industries, Ltd. Osaka Japan insulated cable comparative example versus FEP with 15% SIDISTAR® T 120 insulated cable example of the invention 1. The testing procedure includes the following steps:
1. A six inch piece of Category 5e cable, manufactured to DS-7294, jacketed with PVC plenum compound VP-7 103 and insulated with FEP was suspended approximately 3 inches above a Bunsen burner. This placed the end of the cable in the highest heat area of the flame cone.
2. The Bunsen burner was ignited and a stop watch was begun simultaneously until the first drip was observed and recorded.
3. In addition, the total number of drips during a 2 minute period was recorded.
4. This test was repeated on a six inch piece of Category 5e cable, manufactured to the same specification and using the same jacketing compound. The only difference is this cable was insulated with the FEP/15% SIDISTAR compound.
5. The test was repeated a minimum of five times for each of the two types of samples.
The results are as follows showing that the composite insulation did not drip during a two minute test period:
Results:

**FEP Insulated**

| Trial # | Time to First Drip | Total # of Drips in 2 minutes |
|---|---|---|
| 1 | 0:47 | 39 |
| 2 | 0:54 | 28 |
| 3 | 0:59 | 20 |
| 4 | 0:46 | 37 |
| 5 | 0:42 | 35 |
| 6 | 0:44 | 33 |
| 7 | 0:42 | 43 |
| Average | 0:48 | 33.6 |

**FEP/15% Sidistar Insulated**

| Trial # | Time to First Drip | Total # of Drips in 2 minutes |
|---|---|---|
| 1 | Never | 0 |
| 2 | Never | 0 |
| 3 | Never | 0 |
| 4 | Never | 0 |
| 5 | Never | 0 |
| | | |

Conclusion: The cable insulated with the FEP/15% Sidistar compound never dripped during the two minute test period.

### Testing (flame)

The composite insulation was flame tested according to NFPA262/ UL910 along with a comparative example like the comparative example described above with respect to the drip testing. The amount of bare conductor is measured and reported as flame spread. The composite material of the present invention showed lower flame spread and lower smoke generation than the comparative example.

Referring to Figure 1, the composition insulation in accordance with exemplary embodiments of the present invention may be used for various cable components including but not limited to insulation for the conductors' insulation 120, the cable jacket 110, a separator 130, and the like. Figure 1 shows a cable 100 in accordance with an exemplary embodiment of the present invention including a plurality of paired insulated conductors 140, the separator 130, and the surrounding jacket 110. As used herein "conductor" may be wire, for data or power, or optical fiber. The cable may include other components, such as a metallic shield which may be a braided conductor, a metallic foil, or both, and a barrier layer of insulation disposed between the conductors and the shield.

As seen in Figure 1, the composite insulation with added micro oxide particles of the present invention is preferably used as an insulating layer 120 that insulates the individual conductors 150 of the cable with such conductors typically being twisted into a plurality of pairs, as is known in the art. Although it is preferable that the conductors are twisted together, the conductors may be linearly arranged, i.e. not twisted, either in pairs or groups. Alternatively, a pair of conductors may have intermittent segments that are twisted together. A preferred lay length for twisted conductors or segments thereof is approximately 0.050 to 12 inches.

A conductor insulated with the layer of composite insulation preferably has a dissipation factor of about 0.002 to 0.0002 at 1 GHz when the micro oxide particles, particularly silicon dioxide, are about 5% by weight of the composite, for example. Adhesion to the conductor is increased by about 1% or more than if the conductor is insulated with conventional material. Also, addition of the micro oxide particles allows the insulation to be pressure extruded unlike conventional insulated conductors.

The impedance of a twisted pair is related to several parameters including the diameter of the conductors, the center-to-center distance between the conductors, the dielectric constant of insulating layers, etc. The center-to-center distance is proportional to the thickness of the insulating layers and the dielectric constant depends in part on the properties of the insulation material. The type of micro oxide particles used in the insulating layers may be selected such that insulating layers achieve a desired effective dielectric constant. The concentration of the micro oxide particles embedded in the insulating layer may be controlled so as to control the effective dielectric constant of the resulting composite insulating layer. Accordingly, the dielectric constant may be reduced and/or tailored to meet the requirements of a particular design. Reduced dielectric constants for insulated conductors may yield higher transmission propagation speeds and have generally desirable skew characteristics. In general, it is to be appreciated that micro oxide particles may be used to tailor any characteristic of the cable, such as, but not limited to, characteristic impedance, burn characteristics, skew, crosstalk, and the like.

Moreover, it is to be appreciated that the composite insulation of the present invention may be used to insulate only a single conductor or a pair, more than one conductor or pair, or all of the pairs of the cable, e.g. a 3X1 or 2X2, etc. construction. For example, although Figure 1 shows all of the wire pairs having insulation layers formed of the composite insulation of the present invention, only a single pair may have insulation layers formed of the composite insulation of the present invention with the remaining pairs having insulating layers formed of conventional materials, such as FEP, i.e. a 3X1 construction.

By using the composite insulation of the present invention to insulate a pair of conductors, the impedance of that conductor pair is raised by 0.5 to 10%, the mutual capacitance is lowered by 0.5 to 10%, the velocity of propagation is 0.5 to 30% lower, the difference in the magnitudes of the impedance from the average as swept across a frequency range of 1 Mhz to 2 Mhz is 0.5 to 30% more consistent, the inductance is lowered 0.5 to 10%, the conductance is increased by 0.5 to 10%, and attenuation is improved by more than 1%, as compared to a conductor pair insulated with material without the micro particles of the present invention. The differences reduce the costs of making the insulation and cable and also improve the performance of the cable.

With a plurality of pairs in the cable insulated with the composite insulation of the present invention, the amount of concentration of the micro oxide particles may vary within the pairs of conductors so that the resulting difference signal delay with the pairs is < 25ns (low skew cable). Also, the pairs may be constructed of materials which vary in dielectric constant (PVC olefins, fluoropolymers) and the concentration of silicon dioxide may be varied within the different pairs with that difference resulting in signal delay that is below about 45ns (e.g. 3X1, 2X2 arrangement). It is preferred that the peak optical density (i.e. smoke density) is < 0.5 and that the average optical density is < 0.15 when tested to NFPA 262. This relates to the smoke density of the sample being burned.

Additionally, the conductors 150 of the cable may have dual or more than one layer of insulation where one layer 160 is formed using the composite insulation of the present invention and the other layer 170 is formed using either a conventional material, such as FEP, as seen in Figure 2. Figure 2 shows an exemplary conductor pair 140 where the outer layer 160 is preferably formed of the composite insulation of the present invention and the inner layer 170 is formed of a conventional material. The reverse may also be used. Alternatively, both layers 160 and 170 may be formed using the composite insulation of the present invention. And each layer may have the same or different amounts (percentage of concentration) of the micro oxide particles as compared to the other layer. Moreover, each layer of insulation may be formed using the same or different thermoplastic polymer.

For twisted wire pair applications, the conductors of the pairs may have the same insulation layers or different insulation layers. For example, the dual layers of one conductor of the pair may be both formed of the composite insulation or only one layer may be formed of a conventional material and the same being true of the other conductor of the pair.

The separator 130, as seen in Figure 1, is preferably used to separate the pairs or groups of conductors, as is well known in the art. The separator 130 may be formed linearly along the length of the cable and may have any known shape, such as a cross web or a star. The separator 130 may also be formed with the composite insulation of the present invention. Preferably, the separator 130 is made of a thermoplastic with 1-50% silicon dioxide. The thermoplastic of the separator 130 may be embossed or perforated. The separator 130 may also be foamed up to 50% to reduce material cost. The separator 130 may be embedded with metallic shield segments. The separator 130 may also be formed as bunched fibrillated fibers (i.e. stuffing).

According to another embodiment of the present invention, some of the micro oxide particles of the composite insulation may have a color property. That allows the insulation to have brighter colors. Moreover, the composite insulation creates a surface that print ink will adhere to easily. That allows printing directly on the composite insulation without the need of an additional layer to protect the surface or use of a laser printer. Also, the surface of the composite insulation may be treated with a coupling agent, such as silane, stearic acid, and the like. That improves physical properties and/or allows the addition of a higher level of filler to reduce coat. The composite insulation may contain stabilizers for reducing degradation during processing.

While particular embodiments have been chosen to illustrate the invention, it will be understood by those skilled in the art that various changes and modifications can be made therein without departing from the scope of the invention as defined in the appended claims.
Further features, aspects and embodiments are provided below in the following clauses:
Clause 1. A composite insulation, comprising
   an insulating material; and
   amorphous micro oxide particles added to said insulating material by at least 1% weight of the composition insulation wherein said micro oxide particles provide at least one of an increase in the flame retardancy of the insulating material, a reduction in smoke generated, and an improvement in the electrical properties of the insulating material.
Clause 2. A composite insulation according to clause 1, wherein
   said micro oxide particles are non-porous.
Clause 3. A composite insulation according to clause 2, wherein
   said micro oxide particles are silicon dioxide composite insulation.
Clause 4. A composite insulation according to clause 3, wherein
   said silicon dioxide is up to 80% by weight of the composite insulation.
Clause 5. A composite insulation according to clause 1, wherein
   the dielectric constant of the composite insulation is about 3-30% higher than the insulating material.
Clause 6. A composite insulation according to clause 1, wherein
   the viscosity of the composite insulation is about 3-30% higher than the insulating material.
Clause 7. A composite insulation according to clause 1, wherein
   the melt flow index of the composite insulation is about 3-30% higher than the insulating material.
Clause 8. A composite insulation according to clause 1, wherein
   the melting point of the composition insulation is about 3-50% higher than the insulating material.
Clause 9. A composite insulation according to clause 1, wherein
   the composite material is about 3-30% less translucent than the insulating material.
Clause 10. A composite insulation according to clause 1, wherein
   0.5-10% coloring agent uses about 3-30% less color concentrate in the composite insulation to achieve the same color values than the insulating material with the same percentage of coloring agent.
Clause 11. A composite insulation according to clause 1, wherein
   the charring of the composite insulation is about 3-30% higher than the insulating material.
Clause 12. A composite insulation according to clause 1, wherein
   the composite insulation has a melting point of less than about 270°C.
Clause 13. A composite insulation according to clause 1, wherein
   the micro oxide particles have a mean particle size of about 100 - 300 nm and a mean surface area of less than or equal to about 40 m²/g.
Clause 14. A composite insulation according to clause 1, wherein
   the composite insulation has a dielectric constant of less than 2.4.
Clause 15. A composite insulation according to clause 1, wherein
   the composite insulation exhibits less smoke when burned that the insulating material.
Clause 16. A composite insulation according to clause 1, wherein
   said insulating material is one of polyolefin, polyester, fluoropolymer, Halar, PTFE, PVC, HDPE, and EVA.
Clause 17. A composite insulation according to clause 16, wherein
   said insulation material does not include a polyamide.
Clause 18. An insulated conductor, comprising
   a conductor; and
   at least one layer of a composite insulation surrounding said conductor, said composite insulation including insulating material and micro oxide particles adapted to provide at least one of an increase in the flame retardancy of the insulating material and an improvement in the electrical properties of the insulating material.
Clause 19. An insulated conductor according to clause 18, wherein
   said micro oxide particles is silicon dioxide.
Clause 20. An insulated conductor according to clause 18, wherein
   said micro oxide particles are at least 1% by weight of the composition insulation.
Clause 21. An insulated conductor according to clause 18, wherein
   the dielectric constant and the limiting oxygen index of said composite insulation is about 3-30% higher than the insulation material.
Clause 22. An insulated conductor according to clause 18, wherein
   the viscosity, the melt flow index, and the charring of said composite insulation is about 3-50% higher than the insulating material.
Clause 23. An insulated conductor according to clause 18, wherein
   the insulated conductor has a dissipation factor of about 0.01 to 0.0002 at 1 GHz.
Clause 24. An insulated conductor according to clause 18, wherein
   the adhesion of said composite insulation is higher than the insulating material.
Clause 25. An insulated conductor according to clause 18, wherein
   said composite insulation is at least 5 to 50 % foam.
Clause 26. An insulated conductor according to clause 18, further comprising
   a second layer of insulation surrounding said conductor.
Clause 27. An insulated conductor according to clause 26, wherein
   said second layer of insulation being formed of said composite insulation.
Clause 28. An insulated conductor according to clause 27, wherein
   said at least one layer and said second layer of composite insulation have different amounts of said micro oxide particles in the respective layers.
Clause 29. An insulated conductor according to clause 26, wherein
   said second layer is either an inner or outer layer surrounding said conductor.
Clause 30. An insulated conductor according to clause 26, wherein
   said at least one layer of composite insulation and said second layer of insulation are formed with different thermoplastic polymers.
Clause 31. An insulated conductor according to clause 26, wherein
   either or both of said at least one layer of composite insulation and said second layer of insulation are foamed from about 5 - 50%.
Clause 32. A cable, comprising:
   at least a first pair of conductors;
   at least one of said first pair of conductors having at least one layer of a composite insulation surrounding said conductor, said composite insulation including insulating material and micro oxide particles adapted to provide an increase in the flame retardancy of the insulating material and an improvement in the electrical performance of the cable,
   whereby said conductors of said first pair of conductors may be either twisted together or not twisted together.
Clause 33. A cable according to clause 32, wherein
   said micro oxide particles are silicon dioxide.
Clause 34. A cable according to clause 33, wherein
   said silicon dioxide is at least 1% by weight of the composite insulation.
Clause 35. A cable according to clause 33, wherein
   said silicon dioxide is between about 1% to 80% by weight of the composite insulation.
Clause 36. A cable according to clause 32, wherein
   the micro oxide particles have a mean particle size of about 100 - 300 nm and a mean surface area of less than or equal to about 40 m²/g.
Clause 37. A cable according to clause 32, wherein
   said insulating material is one of polyolefin, polyester, fluoropolymer, Halar, PTFE, PVC, HDPE and EVA.
Clause 38. A cable according to clause 37, wherein
   said insulation material does not include a polyamide.
Clause 39. A cable according to clause 32, wherein
   the dielectric constant and the limiting oxygen index of said composite insulation is about 3-30% higher than the insulation material.
Clause 40. A cable according to clause 32, wherein
   the viscosity, the melt flow index, and the charring of said composite insulation is about 3-50% higher than the insulating material.
Clause 41. A cable according to clause 32, wherein
   said composite insulation is about 5 to 50 % foam.
Clause 42. A cable according to clause 32, further comprising
   a second layer of insulation surrounding said conductor of said first pair of conductors that has the at least one layer of a composite insulation.
Clause 43. A cable according to clause 42, wherein
   said second layer of insulation is formed of said composite insulation.
Clause 44. A cable according to clause 42, wherein
   said at least one layer and said second layer of composite insulation have different amounts of said micro oxide particles in the respective layers.
Clause 45. A cable according to clause 42, wherein
   said at least one layer of composite insulation and said second layer of insulation are formed with different thermoplastic polymers.
Clause 46. A cable according to clause 32, wherein
   said conductors are twisted with a lay length of about 0.050 to 12 inches.
Clause 47. A cable according to clause 32, further comprising
   a second pair of conductors, each of said conductors of said second pair of conductors having a layer formed of an insulating material.
Clause 48. A cable according to clause 47, wherein
   both of the conductors of said first pair of conductors having a layer of insulation formed of said composite material,
   whereby the impedance of said first pair of conductors is 0.55 to 10% higher, the mutual capacitance is 0.55 to 10% lower, the velocity of propagation is 0.5% to 30% lower, the difference in the magnitudes of the impedance from the average as swept across a frequency range of 1 MHz to 2 MHz is 0.5 to 30% more consistent, the inductance is 0.5% to 10% lower, the conductance is 0.5 to 10% higher, and attenuation is improved by more than 1%, as compared to said second pair of conductors.
Clause 49. A cable according to clause 48, wherein
   the amount of micro oxide particles in the composite insulation of said first pair of conductors differs from the amount of micro oxide particles in the composite insulation of said second pair of conductors.
Clause 50. A cable according to clause 48, wherein
   said first and second pairs of conductors are twisted with an overall cable lay of about 0.5 to 36 inches.
Clause 51. A cable according to clause 48, wherein
   the amount of concentration of the micro oxide particles varies within the composite insulation of the first and second pairs of conductors so that the resulting difference signal delay with the pairs is < 25ns.
Clause 52. A cable according to clause 48, wherein
   the composite insulation of said first and second pairs are constructed of materials which vary in dielectric constant and the concentration of the micro oxide particles is varied with in the different pairs resulting in signal delay that is below 45ns.
Clause 53. A cable according to clause 48, wherein
   the peak optical density of the cable is about less than 0.5, and the average optical density of the cable is less than 0.15 when tested to NFPA 262.
Clause 54. A cable according to clause 48, further comprising
   at least one of a jacket for enclosing said first and second pairs of conductors and a separator for separating said first and second pairs of conductors, wherein at least one of said jacket and said separator is formed of said composite insulation.
Clause 55. A cable, comprising:
   a plurality of conductors, each conductor being surrounded by a layer of insulating material;
   a jacket enclosing said plurality of conductors, said jacket being formed of an insulating material; and
   a separator separating said plurality of conductors, said separator being formed of an insulating material,
   whereby said insulation material of at least one of said plurality of conductors, said jacket, and said separator including micro oxide particles to form a composite insulation which has at least one of an increased flame retardancy and improved electrical properties over the insulating material without the micro oxide particles, such that the cable has an improved electrical performance.
Clause 56. A cable according to clause 55, wherein
   said micro oxide particles are silicon dioxide.
Clause 57. A cable according to clause 56, wherein
   said silicon dioxide is at least 1% by weight of the composite insulation.
Clause 58. A cable according to clause 55, wherein
   the micro oxide particles have a mean particle size of about 100 - 300 nm and a mean surface area of less than or equal to about 40 m²/g.
Clause 59. A cable according to clause 55, wherein
   the insulating material is one of polyolefin, polyester, fluoropolymer, Halar, PTFE, PVC, HDPE and EVA.
Clause 60. A cable according to clause 59, wherein
   the insulation material does not include a polyamide.
Clause 61. A cable according to clause 55, wherein
   the insulating material of each of said layers of said plurality of conductors, said jacket, and said separator is formed of said composite insulation.
Clause 62. A cable according to clause 55, wherein
   said composite insulation is about 5 to 50 % foam.
Clause 63. A cable according to clause 55, further comprising
   a second layer of insulation surrounding at least one of said of said plurality of conductors, said second layer being formed of said composite insulation.
Clause 64. A cable according to clause 63, wherein
   both of said layers of said conductors are formed of said composite insulation.
Clause 65. A cable according to clause 63, wherein
   said layers of composite insulations are formed with different thermoplastic polymers.
Clause 66. A cable according to clause 55, wherein
   said plurality of conductors are twisted into a plurality of pairs of conductors whereby said separator separate said plurality of pairs.
Clause 67. A cable according to clause 65, wherein
   at least one of said plurality of pairs of conductors having layers of insulation formed with said composite insulation.
Clause 68. A cable according to clause 55, further comprising
   a metallic shield encompassing said plurality of conductors.
Clause 69. A cable according to clause 68, wherein
   said metallic shield is one of a braided conductor, metallic foil, or both.
Clause 70. A cable according to clause 55, wherein
   said insulating material of said separator is a thermoplastic with 1-50% silicon dioxide.
Clause 71. A cable according to clause 55, wherein
   said separator is formed linearly along the length of the cable to separate conductors.
Clause 72. A cable according to clause 55, wherein
   said separator is foamed up to 50%.
Clause 73. A cable according to clause 55, wherein
   said separator is embossed or perforated.
Clause 74. A cable according to clause 55, wherein
   said separator is in the form of flakes or dielectric segments.
Clause 75. A cable according to clause 55, wherein
   said separator is embedded with metallic shield segments.
Clause 76. A cable according to clause 55, wherein
   said separator is formed into bunched fibrillated fibers.
Clause 77. A cable according to clause 55, further comprising
   a barrier layer of insulation disposed between said plurality of conductors and a metallic shield.
Clause 78. A cable according to clause 55, wherein
   said jacket is formed of said composite material.
Clause 79. A cable according to clause 78, wherein
   said jacket is formed of fluoropolymer with at least 1% silicon dioxide.
Clause 80. A cable according to clause 78, wherein
   said jacket surface is suitable for the application of printer ink.
Clause 81. A composite insulation for a cable component, comprising
   an insulating material; and
   solid, non-porous, low surface area, non-ionic, non-hydrated, mineral or metal micro oxide particles added to said insulating material by at least 1% weight of the composition insulation wherein said micro oxide particles increase the flame retardancy of the insulating material and improve the electrical performance of the cable.
Clause 82. A composite insulation according to clause 81, wherein said micro oxide
   particles are silicon dioxide.
Clause 83. A composite insulation according to clause 82, wherein said insulation material does not include a polyamide.

## Claims

1. An insulated conductor, comprising
a conductor; and
at least one layer of a composite insulation surrounding said conductor, said composite insulation including insulating material and micro oxide particles adapted to provide at least one of an increase in the flame retardancy of the insulating material and an improvement in the electrical properties of the insulating material.

2. An insulated conductor according to claim 1, wherein
said micro oxide particles is silicon dioxide.

3. An insulated conductor according to claim 1, wherein
said micro oxide particles are at least 1% by weight of the composition insulation.

4. An insulated conductor according to claim 1, wherein
the dielectric constant and the limiting oxygen index of said composite insulation is about 3-30% higher than the insulation material.

5. An insulated conductor according to claim 1, wherein
the viscosity, the melt flow index, and the charring of said composite insulation is about 3-50% higher than the insulating material.

6. An insulated conductor according to claim 1, wherein
the insulated conductor has a dissipation factor of about 0.01 to 0.0002 at 1 GHz.

7. An insulated conductor according to claim 1, wherein
the adhesion of said composite insulation is higher than the insulating material.

8. An insulated conductor according to claim 1, wherein
said composite insulation is at least 5 to 50 % foam.

9. An insulated conductor according to claim 1, further comprising
a second layer of insulation surrounding said conductor.

10. An insulated conductor according to claim 9, wherein
said second layer of insulation being formed of said composite insulation.

11. An insulated conductor according to claim 10, wherein
said at least one layer and said second layer of composite insulation have different amounts of said micro oxide particles in the respective layers.

12. An insulated conductor according to claim 9, wherein
said second layer is either an inner or outer layer surrounding said conductor.

13. An insulated conductor according to claim 9, wherein
said at least one layer of composite insulation and said second layer of insulation are formed with different thermoplastic polymers.

14. An insulated conductor according to claim 9, wherein
either or both of said at least one layer of composite insulation and said second layer of insulation are foamed from about 5 - 50%.
